

No. 711,835.

Patented Oct. 21, 1902.

M. DUCAT, C. J. A. MARNAS & L. H. DEHOFF.

PROCESS OF SILK PRINTING.

(Application filed Sept. 6, 1900.)

(No Model.)

Fig. 1.



Fig. 2.



glossy



dull

WITNESSES:

Bernhard C. Hesse.  
Chas. E. Preusser.

INVENTORS:

M. Ducat  
C. J. A. Marnas  
L. H. Dehoff

BY Hauff & Hauff

ATTORNEYS

# UNITED STATES PATENT OFFICE.

MATHIEU DUCAT, OF NEUVILLE-SUR-SAÔNE, AND CHARLES JEAN ANTOINE MARNAS, OF LYONS, FRANCE, AND LEOPOLD HEINRICH DEHOFF, OF LUDWIGSHAFEN, GERMANY, ASSIGNORS TO THE BADISCHE ANILIN & SODA FABRIK, OF LUDWIGSHAFEN, GERMANY, A CORPORATION.

## PROCESS OF SILK-PRINTING.

SPECIFICATION forming part of Letters Patent No. 711,835, dated October 21, 1902.

Application filed September 6, 1900. Serial No. 29,182. (No specimens.)

*To all whom it may concern:*

Be it known that we, MATHIEU DUCAT, dyer, residing at Neuville-sur-Saône, and CHARLES JEAN ANTOINE MARNAS, dyer, residing at 5 Lyons, France, citizens of the French Republic, and LEOPOLD HEINRICH DEHOFF, doctor of philosophy and chemist, a subject of the King of Saxony, residing at Ludwigshafen-on-the-Rhine, in the Kingdom of Bavaria, Germany, have invented a new Process of Silk-Printing, of which the following is a specification.

The object of this invention is to obtain prints consisting of a dull background and a 15 glossy design or the reverse on fabric consisting of or containing raw silk. Such patterns have hitherto been obtained only by weaving together raw and degummed silk in appropriate manner, and consequently in such fabric the separate and individual threads each consist entirely of either raw or degummed silk. Now we have discovered that patterns of this kind can be obtained by locally degumming the raw silk, and this may be accomplished by printing the design by means 20 of a paste containing a caustic alkali—for instance, caustic soda—and then subjecting the so-printed material to proper subsequent treatment; but we have also found that unless great care be exercised in this process the 25 action of the caustic alkali is very apt to go beyond the mere removal of the silk-gum and to attack the silk fiber itself, thus reducing its strength. We have further discovered that this action of the caustic alkali can be 30 so modified that the gum is removed and the strength of the silk fiber is not affected. This we do by adding to the degumming-paste some such substance as will limit the action of the 35 paste to the gum. We have found that grape-sugar or glycerin possesses this property, and therefore a suitable paste can be made by adding to the caustic-soda paste grape-sugar or glycerin. In the following we will refer to 40 grape-sugar or glycerin as "limiting agent." 45 For our purpose we can use either dyed or undyed fabric. If the fabric is dyed and the

shade of the printed goods is to remain unimpaired, then it is evident that the coloring-matter in the dyed fabric employed must be 50 indifferent to the action of the degumming-paste. Similarly the above printing-paste may also contain such color-matter or coloring-matters as are not affected by the degumming-paste, when glossy colored designs 55 will be obtained on a dull background, or vice versa. We have also discovered that indigo, anthraquinone black, oxamin red, &c., are suitable for this purpose. Further, we have also discovered that the above-mentioned designs can be made on silk fabric by printing such reserves on the fabric, which when dried or steamed are indifferent to the action of alkali, and by then passing the so-printed fabric through a bath containing caustic alkali, such as caustic soda, and a substance which will limit the action of the bath to the silk-gum, such as grape-sugar or glycerin. Among such reserves we may mention 60 chrome acetate. The reserves likewise may 65 contain appropriate coloring-matter.

In the following examples we illustrate the nature of our invention and how it may best be carried into effect; but we do not wish to be understood as limiting our invention to 70 these examples. The parts are by weight:

*Example 1—Printing a degumming-paste containing caustic soda.*—Make a paste of two hundred (200) parts of British gum and four hundred (400) parts of hot water. Cool and 80 add four hundred (400) parts of caustic-soda solution of forty (40°) degrees Baumé. Print this paste upon dyed or undyed raw silk, dry at a moderate temperature—say thirty-five (35°) degrees centigrade—rinse, and, if 85 desirable, pass through an acid-bath. The so-prepared material can be dyed in the usual manner, if desired.

*Example 2—Printing a degumming-paste containing caustic soda and a limiting agent.*— 90 Introduce one hundred (100) parts of British gum in the usual manner into seven hundred (700) parts of caustic-soda solution of forty (40°) degrees Baumé. Prepare also a mixture

of three hundred (300) parts of grape-sugar in one hundred (100) parts of water by heating on a water-bath, stir until cool, and pour into the British gum caustic-soda paste and bring up

5 to twelve hundred (1,200) parts by addition of water, if necessary. Print this paste and finish the material as in Example 1.

*Example 3—Printing a degumming-paste containing caustic soda, a limiting agent, and 10 a coloring-matter.*—(A) Make a paste of ten (10) parts of anthraquinone black and forty (40) parts of cold water; also, mix sixty (60) parts of British gum with seven hundred (700) parts of caustic-soda solution of forty (40°) degrees 15 Baumé, and add to this, as in Example 2, three hundred (300) parts of grape-sugar mixed with ninety (90) parts of water. Mix all these and bring up to twelve hundred (1,200) parts by addition of water, if necessary. Print and finish as in Example 1.

(B) Introduce sixty (60) parts of British gum into seven hundred (700) parts of caustic-soda solution of forty (40°) degrees Baumé. Add thirty (30) parts of indigo J. Prepare 25 also a mixture of three hundred (300) parts of grape-sugar and one hundred (100) parts of water by heating on a water-bath. Stir until cool and pour into the British gum indigo J and caustic-soda paste and bring up to twelve 30 hundred (1,200) parts by addition of water, if necessary. Print this paste and finish the material as in Example 1.

*Example 4—Printing a reserve and locally degumming by means of caustic soda and a limiting agent.*—Mix five hundred and fifty (550) parts of hot water with three hundred (300) parts of British gum. Cool and add one hundred and fifty (150) parts of a solution of chrome acetate of twenty (20°) degrees Baumé and make up to one thousand (1,000) parts by addition of water. Print this paste onto the material, dry, and then pass through a bath containing three hundred (300) parts of glycerin, two hundred (200) 45 parts of water, seven hundred (700) parts of caustic-soda solution of forty (40°) degrees

Baumé for from two (2) to five (5) minutes. Then rinse well in running water.

In the annexed drawings are shown two pieces of silk.

In Figure 1 the body or main part of the piece is glossy, while a part thereof—say a flower or any other figure—is dull, while in Fig. 2 the main part of the piece of silk is dull and a portion is glossy.

What is claimed is—

1. As a new article of manufacture, fabric containing locally-degummed silk.

2. As a new article of manufacture, fabric containing locally-degummed silk whereby a 60 surface design is produced.

3. The process of locally degumming silk which consists in the application of caustic alkali and a limiting agent to part only of un-degummed silk.

4. The process of locally degumming silk which consists in the application of caustic alkali to part only of undegummed silk.

5. The process of locally degumming silk which consists in the application of caustic 70 soda and a limiting agent to part only of un-degummed silk.

6. The process of locally degumming silk, which consists in the application of caustic soda and grape-sugar to part only of undegummed silk.

7. The process of locally degumming silk which consists in the application of caustic soda to part only of undegummed silk.

In testimony whereof we have hereunto set 80 our hands in the presence of two subscribing witnesses.

MATHIEU DUCAT.

CHARLES JEAN ANTOINE MARNAS.

LEOPOLD HEINRICH DEHOFF.

Witnesses for Ducat and Marnas:

HUMBERT LOUIS,

ANTOINE S. LOCHEL.

Witnesses for Leopold Heinrich Dehoff:

ERNEST G. EHRHARDT,

JACOB ADRIAN.